

Aug. 29, 1939.

D. H. WAMSLEY

2,171,230

INSULATING COATING

Filed Feb. 28, 1938

*Fig. 1*



*Fig. 2*



BY

INVENTOR.  
DELOS H. WAMSLEY

*Charles M. Clark*  
ATTORNEY.

## UNITED STATES PATENT OFFICE

2,171,230

## INSULATING COATING

Delos H. Wamsley, West Caldwell, N. J., assignor,  
by mesne assignments, to Radio Corporation of  
America, New York, N. Y., a corporation of  
Delaware

Application February 28, 1938, Serial No. 193,137

4 Claims. (Cl. 250—177)

My invention relates to electron discharge devices, and to means for substantially eliminating secondary electron emission from the surfaces in such tubes exposed to primary electron bombardment, and particularly to the prevention of secondary electron emission from and surface leakage along insulators and insulating spacers for electrodes in such devices.

It is common practice to use mica or ceramic spacers in electrode mounts to insulatingly space the electrodes. It has been proposed to coat the insulating surfaces of envelopes and spacers of radio tubes with powdered refractory metal compounds to increase the effective electrical distance between points on the surface and thereby reduce leakage. The compounds heretofore used for such coating are ineffective in preventing secondary electron emission from the coated surface.

20 An object of my invention is to provide coating material to reduce direct leakage over the surfaces of insulators, such as spacers, and which also prevents electron emission from the coated surfaces.

25 A better understanding of my invention may be obtained by referring to the following specification in which preferred embodiments are described for purposes of illustration.

Figure 1 represents a conventional tube with 30 insulating surfaces coated with a layer of an alumina hydrate according to my invention and Figure 2 shows an enlarged view of an insulator for an electron discharge device coated in accordance with my invention with an alumina hydrate.

For purposes of illustrating my invention an electron discharge device with a conventional glass envelope 1 is shown enclosing any desired electrode arrangement including a cathode 2. Insulating surfaces of the envelope and of mica spacers 3 and 4 are coated with a material 5 for reducing secondary emission. The coating as shown in Figure 2 may be applied in an adherent uniform layer on any of the insulator surfaces which may receive electrons from the cathode.

Insulating surfaces of an electron discharge device including the surfaces between metal conductors of different potentials, such as the envelope wall adjacent the lead-in seals, grids, and electrode spacers of the mica or ceramic type, as well as grids and metal parts are coated, according to my invention, with a layer of alumina monohydrate,  $\text{Al}_2\text{O}_3\text{—H}_2\text{O}$ . The alumina monohydrate is preferably powdered to a particle size

of less than 50 microns, and suspended in water or in a volatile liquid, such as nitrocellulose. The suspension may be applied to the surfaces by spraying, dipping or painting and the surfaces dried to leave on them a rough adherent coating 5 of alumina monohydrate. It has been found that a coating approximately .005" thick on the surfaces will suppress secondary electron emission and will also prevent leakage over insulators or insulating surfaces, such as the mica spacer in 10 the conventional type of tube shown for example in United States Patent 1,672,233 to Skinner. The coated parts are assembled in the electron discharge device and during exhaust the parts are heated in the usual manner to drive out 15 occluded gases.

An electron discharge device constructed in accordance with my invention has practically no secondary electron emission from the coated surfaces, and has very low leakage currents over 20 its insulating surfaces between conductors of different potentials. The operation of my tube in high frequency currents is particularly stable because of the absence of emission of secondary electrons from surfaces coated with my novel 25 insulating coating material.

I have found that alumina monohydrate coated on insulating surfaces not only practically eliminates secondary electron emission from the surfaces, but also substantially reduces leakage 30 currents over the surfaces, particularly in tubes having cathodes coated with barium and strontium oxides. In such tubes it seems probable that active metals, such as barium, often evaporate from getters or the oxide coated cathode 35 and condense on insulating surfaces in the usual electron discharge device, producing troublesome leakage paths and sources of secondary electrons on the surfaces. It is my belief that alumina monohydrate coated on insulating surfaces 40 in accordance with my invention reacts with the active metals condensed thereon to form inert compounds which are resistive to leakage currents and prevent emission of secondary electrons. Tests indicate, and it is my belief, that 45 alumina monohydrate coated on the insulating surfaces in accordance with my invention retains its water of crystallization during manufacture and exhaust of the electron discharge device. Barium depositing on the alumina monohydrate is probably converted into barium hydroxide, which is an effective insulator for leakage currents and is particularly inert as a source of secondary electrons. As alumina monohydrate 50 is a crystalline material, which when sprayed 55

and dried forms a roughened granular coating, the reduction in leakage is apparently due to an increase in length of leakage paths over the surface.

5 I claim:

1. An electron discharge device having cooperating electrodes in an envelope, insulating surfaces in said envelope, and a coating of alumina monohydrate at least .005" thick on said surfaces.
- 10 2. An electron discharge device, an insulator in said device, and a coating of alumina monohydrate on the surface of said insulator.
3. An electron discharge device comprising an

envelope and cooperating electrodes in said envelope, a coating of an alumina hydrate on insulating surfaces in said envelope to reduce leakage currents over and secondary emission from said surfaces.

5 4. An electron discharge device with an envelope containing an oxide coated cathode and cooperating electrodes, comprising means for preventing emission of secondary electrons from some of the surfaces in the envelope of said 10 electron discharge device comprising a coating of alumina monohydrate on said surfaces.

DELOS H. WAMSLEY.